

L. T. FREDERICK & L. McCULLOCH,  
MAGNETIC MATERIAL,  
APPLICATION FILED JAN. 7, 1914.

1,231,588.

Patented July 3, 1917.

Fig. 9.



Fig. 8.



Fig. 7.



Fig. 6.



Fig. 5.



Fig. 4.



Fig. 3.



Fig. 2.



Fig. 1.



WITNESSES:

Y Fred H. Miller  
R. D. Brown

INVENTORS  
Louis T. Frederick  
& Leon McCulloch  
BY Wesley Glass  
ATTORNEY

# UNITED STATES PATENT OFFICE.

LOUIS T. FREDERICK AND LEON McCULLOCH, OF WILKINSBURG, PENNSYLVANIA,  
ASSIGNORS TO WESTINGHOUSE ELECTRIC AND MANUFACTURING COMPANY, A  
CORPORATION OF PENNSYLVANIA.

## MAGNETIC MATERIAL.

1,231,588.

Specification of Letters Patent.

Patented July 3, 1917.

Application filed January 7, 1914. Serial No. 810,872.

*To all whom it may concern:*

Be it known that we, LOUIS T. FREDERICK, a citizen of the United States, and a resident of Wilkinsburg, in the county of Allegheny and State of Pennsylvania, and LEON McCULLOCH, a citizen of the United States, and a resident of Wilkinsburg, in the county of Allegheny and State of Pennsylvania, have invented a new and useful Improvement in 10 Magnetic Material, of which the following is a specification.

Our invention relates to the manufacture of magnetic material, and it has particular reference to the manufacture of such material to be formed into wedges for use in the slots of dynamo-electric machines.

In induction motors and other dynamo-electric machines which comprise magnetizable core members having coil-containing slots, it is desirable that the coils be of the partially closed type, since, by the use of this type of coils, eddy currents are minimized and slot leakage decreased, with consequent lowering of the reactance of the machine and a proportional increase in its general efficiency. Furthermore, when the slotted core is the rotor of the machine, the partial closure of the slots serves to hold the coils firmly against centrifugal or other displacement.

On the other hand, the open type of slot having parallel sides is preferable on account of certain mechanical considerations, among which are simplicity of construction and the fact that the coils may be readily reached for removing or repairing them. It has therefore been found desirable to combine the advantages of both types of slots by providing slots of the open type and supplying them with removable wedges of magnetic material. These wedges have heretofore usually been composed of two strips of a magnetic substance, such as iron or steel and a separating strip of non-magnetic substance, such as brass.

It is the object of our invention to provide a cheap and efficient magnetic material from which unitary wedges may be made which will have the same effect as the tripartite wedges heretofore used.

Our invention comprehends our improved magnetic material and the steps of the process by which it is produced.

In general, we proceed by distributing

separate bodies of a magnetic substance 55 throughout a mass of non-magnetic material which serves as a binder and carrier for the magnetic bodies. At suitable intervals, we provide sections composed entirely of non-magnetic material so as to enable 60 wedges to be cut, each of which will include one of these entirely non-magnetic portions to constitute the necessary magnetic gap in the wedge. We have found it convenient to prepare the mass in the form of a laminated 65 fabric having strips, wire or finely divided particles of a magnetic substance, such as iron, disposed between the laminations.

The nature of our invention will be best understood by reference to the accompanying drawings, in which Figure 1 is a fragmentary perspective view showing one manner in which the laminations may be stacked in the first stage of our process; Fig. 2 is a fragmentary perspective view showing an 70 other laminated arrangement built up in accordance with our process; Fig. 3 is a perspective view of a composite sheet formed by pressing the stack of material shown in Fig. 2; Fig. 4 is a view similar to Fig. 3 showing 75 a composite sheet in which metallic ribbons are embedded; Fig. 5 is another view similar to Fig. 3 showing a composite sheet having a finely divided magnetic substance distributed therethrough; Fig. 6 is a view similar 80 to Fig. 4 showing a sheet carrying metallic ribbons which are crimped or plaited at the edges; Fig. 7 is a plan view showing a sheet prepared according to our invention and divided into parallel spaced strips; Fig. 8 is a 85 perspective view showing a portion of a sheet which has been subjected to further treatment according to our invention, and Fig. 9 is an elevational view showing a series of core slots, one of which is provided 90 with one of our improved wedges.

Referring now to Figs. 1 and 2 of the drawing, wires 1 of a magnetic material are laid, woven or stretched parallel to one another. This may be conveniently done by 100 weaving a fabric in which the warp is composed of fine wire and the weft of cotton or similar thread. Such a fabric is shown in Fig. 1, in which the wires 1 are woven with threads 2. The wires or wire-fabric sheets 105 are then sandwiched between sheets of paper or cloth 3—3 treated with a phenolic condensation product or other adhesive insulat-

ing substance and stacked to any desired thickness. Instead of wires, ribbons of iron may be employed as shown at 4, in Fig. 4, and these ribbons may be plaited at the 5 edges, as shown at 5, in Fig. 6. The process may be further modified by employing finely divided iron or other magnetic material as shown at 6, in Fig. 5. In this case, the finely divided magnetic material is sprinkled or 10 otherwise spread uniformly over the paper or cloth after treating the fabric with the adhesive. The stacked material, however prepared, is then placed between clean plates and pressed in a hot press. The sheets 15 formed by pressing the stacked material shown in Figs. 1 and 2 present the appearance shown in Fig. 3. Both surfaces of the pressed sheet are then smoothed and the plate is sawed into parallel strips. Enough 20 material is left at each end of the saw-cuts 7, as shown in Fig. 7, to keep the strips evenly separated from one another. When 25 the magnetic substance is in the form of wire or of ribbon-like strips, the saw-cuts are transverse to the wires or strips, as is clearly shown in Fig. 7. The saw-cuts 7 are then filled with a cement, a cement and a suitable filler, or other cementitious or solid insulating material. Paper or cloth treated 30 with an adhesive, such as a phenolic condensation product or its equivalent, should then be placed on both sides of the spaced strips, which are then placed between clean plates and hot pressed into a solid sheet. Such a 35 sheet is shown in Fig. 8, the outer sheets being designated by 8-8.

In order to form wedges from the material so prepared, the composite sheet is divided by cuts made in the same direction 40 as the cement-filled slots, and the cuts should be so made as to bring the slots approximately in the center of the wedges. For example, a wedge might be formed by cutting along the lines A B and C D of Fig. 7. 45 The wedges should be of a suitable width to be received in the grooves 9 formed near the top of the slots 10 shown in Fig. 9, and their edges are properly shaped to be received in the grooves as shown. 50 Various modifications and changes may be made in the steps of the process and in the arrangement of the parts which make up our improved material without departing from the spirit and intent of our invention, 55 and we wish it to be understood, therefore, that our invention is not restricted to the exact modifications which we have disclosed above, but is limited only by the scope of the appended claims.

60 We claim as our invention:

1. A process of making magnetic material which comprises distributing a plurality of bodies of a magnetic substance upon a sheet of fibrous material which has been coated 65 with an electrically insulating adhesive sub-

stance, stacking a plurality of sheets so treated one upon the other and pressing the stacked material between heated surfaces.

2. A process of making magnetic material which comprises distributing a plurality of strips of a magnetic substance in parallel relation upon a sheet of fibrous material coated with an electrically insulating adhesive substance, stacking a plurality of sheets so treated upon one another and pressing the stacked material between heated surfaces. 75

3. A process of making magnetic material which comprises distributing a plurality of wires of a magnetic substance in parallel 80 relation upon a sheet of fibrous material coated with an electrically insulating adhesive substance, stacking a plurality of sheets so treated upon one another and pressing the stacked material between heated 85 surfaces.

4. A process of making magnetic material which comprises distributing a plurality of bodies of a magnetic substance upon a sheet of fibrous material coated with an electrically insulating adhesive substance, stacking a plurality of sheets so treated one upon another, pressing the stacked material between heated surfaces, smoothing the surfaces of the pressed sheet, cutting the pressed 95 sheet into parallel strips separated by narrow slots, filling the slots with non-magnetic material and inclosing the sheet so treated between sheets of fibrous material. 100

5. The process of making magnetic material which comprises preparing a sheet of non-magnetic material having bodies of magnetic material distributed therethrough, dividing the sheet into spaced parallel strips, filling the spaces between the strips 105 with a non-magnetic material and inclosing the spaced strips between sheets of fibrous material.

6. The process of making magnetic material which comprises preparing a sheet of non-magnetic material having relatively long bodies of magnetic material distributed therethrough, dividing the sheet into spaced parallel strips, filling the spaces between the strips 110 with a non-magnetic material and inclosing the spaced strips between sheets of fibrous material. 115

7. The process of making magnetic material which comprises preparing a sheet of non-magnetic material having bodies of magnetic material distributed therethrough, dividing the sheet into spaced parallel strips, filling the spaces between the strips with a non-magnetic material, inclosing the spaced strips between sheets of fibrous material, 120 and dividing the pressed sheet into strips by cuts parallel to the spaces filled with non-magnetic material. 125

8. A process of making magnetic material which comprises preparing a lami- 130

nated sheet of non-magnetic material having bodies of magnetic material distributed therethrough, dividing the sheet into parallel spaced strips, filling the spaces between the strips with non-magnetic material and pressing the sheet between layers of fibrous material.

9. A process of making magnetic material which comprises preparing a laminated sheet of non-magnetic material having bodies of magnetic material evenly distributed therethrough, dividing the sheets into evenly spaced parallel strips, filling the spaces between the strips with a cement, hot-pressing the spaced strips between two sheets of fibrous material and dividing the sheet into strips by cuts parallel to and spaced from the cement-filled spaces.

10. As a new article of manufacture, magnetic material comprising a laminated sheet of non-magnetic material having bodies of a magnetic substance distributed therethrough.

11. As a new article of manufacture, magnetic material comprising a laminated sheet of non-magnetic material having wires of a magnetic substance distributed therethrough.

12. As a new article of manufacture, magnetic material comprising a sheet of non-magnetic material having bodies of a magnetic substance distributed therethrough and having relatively narrow spaced sections of cement.

13. As a new article of manufacture, a 35 magnetic material comprising a mass of non-magnetic material having a relatively large number of parallel wires of a magnetic substance distributed therethrough, relatively narrow spaced sections of a cement disposed transversely to the wires and extending completely through the mass, and sheets of non-magnetic material inclosing the mass.

14. A wedge for closing core slots of 45 dynamo-electric machines comprising a unitary strip having an intermediate longitudinal section of non-magnetic material and two longitudinal outer sections composed of transversely disposed wires of a magnetic 50 material compressed between laminations of non-magnetic material.

15. A wedge for closing core slots of 55 dynamo-electric machines comprising a unitary strip having an intermediate longitudinal section of non-magnetic material and two longitudinal outer sections composed of laminated non-magnetic material having bodies of a magnetic substance distributed therethrough.

In testimony whereof, we have hereunto subscribed our names this 31st day of Dec., 1913.

LOUIS T. FREDERICK.  
LEON McCULLOCH.

Witnesses:

PHILLIPS THOMAS,  
B. B. HINES.